

# UNITED STATES PATENT OFFICE.

ROMAN v. ZELEWSKI, OF ENGIS, VILLA D'EHEIN, BELGIUM.

PROCESS OF ROASTING ORES, INTERMEDIATE PRODUCTS, AND OTHER METALLIFEROUS MATERIALS.

1,097,500.

Specification of Letters Patent.

Patented May 19, 1914.

No Drawing.

Application filed February 18, 1913. Serial No. 749,233.

*To all whom it may concern:*

Be it known that I, ROMAN v. ZELEWSKI, director, a subject of the King of Prussia, residing at Engis, Villa d'Ehein, in the 5 Kingdom of Belgium, have invented certain new and useful Improvements in Processes of Roasting Ores, Intermediate Products, and other Metalliferous Materials; and I do hereby declare the following to be a 10 full, clear, and exact description of the invention, such as will enable others skilled in the art to which it appertains to make and use the same.

This invention relates to an improved 15 process for roasting ores.

According to my improved process, I propose to refine briquets containing sulfurous ores and intermediate products, the briquets simply being roasted.

20 In carrying out my improved process, briquets containing sulfid ores are piled in checker-board form in an inclosure, and then hot products of combustion to pre-heat and ignite the gases liberated from the bri- 25 quets are supplied. To augment the combustion, air under pressure is introduced to the inclosure, which by reason of the porous character of the briquets, and the fact that the latter are spaced apart, the heat is 30 forced through and around said briquets. After the briquets are heated sufficiently to liberate the gases and the latter become ignited, the heated products of combustion are discontinued, although the supply of air is 35 continued to assist in liberating the gases and promote the combustion. This operation is continued until the combustible gases are consumed and the briquets reach a slag condition, whereupon the supply of air is 40 cut off.

My invention is particularly well adapted

for the treatment of briquets, the constituent parts of which are formed of ores known as blends. These ores contain gaseous fuel which must be eliminated without absorbing 45 the metal, vapors or oxids. I have found that when the ore is made into briquet form and first subjected to pre-heating combustion, with the assistance of air under pressure to liberate the gases, the briquets 50 will roast, and the salient oxids will be preserved.

The briquets are porous, hence when the pre-heating combustion is applied, the air forces the combustion through the pores and 55 drives the combustible gases out, and they become ignited and eventually, with the assistance of the air, complete the roasting process.

Having thus described my invention, 60 what I claim is:

The herein described process of treating briquets containing sulfid ores, consisting in inclosing spaced apart briquets supplying hot products of combustion to preheat and 65 ignite the gases liberated from the heated briquets, discontinuing the supply of heated products of combustion after ignition of the gases has commenced, continuing the supply of air under pressure, causing the same to 70 permeate the pores in the briquets and pass around the latter, and augment the combustion until the combustible gases are consumed and the briquets reach a slag condition, then cutting off the supply of air. 75

In testimony whereof I have signed my name to this specification in the presence of two subscribing witnesses.

ROMAN v. ZELEWSKI.

Witnesses:

A. P. CRUGER,  
L. PARMENTIER.